# EUROPEAN PATENT SPECIFICATION

(11) **EP 0 011 497 B1**
(45) Date of publication and mention of the grant of the patent: **16.02.1983**
(21) Application number: 79302596.6
(22) Date of filing: 15.11.1979
(51) Int. Cl.: C10M 1/24, C23F 11/12

(54) **Lubricating oil composition and additive concentrate for addition to lubricating oil**
Schmierölzusammensetzung und Zusatzkonzentrat für den Zusatz zu Schmieröl
Composition d'huile lubrifiante et concentrat d'additif pour l'addition à de l'huile lubrifiante

(30) Priority: 15.11.1978 US 960764
(43) Date of publication of application: 28.05.1980
(73) Proprietor: EDWIN COOPER INC., St. Louis Missouri 63104 (US)
(72) Inventor: Harstick, Christian S., Crestwood Missouri 63126 (US); Zaweski, Edward F., Pleasant Ridge Michigan 48029 (US)
(74) Representative: Bizley, Richard Edward

## Description

This invention relates to a lubricating oil composition and an additive concentrate for addition to lubricating oil; and the invention is concerned, in particular, with the provision of an improved oil for crankcase service for internal combustion engines. Oils for such service commonly contain various additives which serve different functions. Ashless dispersants are added to prevent deposition of engine sludge. Zinc dihydrocarbyldithiophosphate is added to inhibit wear and provide antioxidant protection. Alkaline earth metal alkylbenzene or petroleum sulfonates function as high temperature detergents. Over-based alkaline earth metal sulfonates or salicylates provide both detergent action and an alkaline reserve to protect engine parts against corrosion.

The use of certain surfactants for lubricating oil is discussed in U.S. Patents Nos. 3,509,052 and 3,928,219. These include certain oxyalkylated polyols, oxyalkylated ethylenediamine, nonylphenyl polyethylene glycol ethers and the like. Furthermore, U.S. Patents Nos. 2,681,315 and 2,833,717 disclose the use of oxyethylated alkylphenols in oil as corrosion inhibitors. In addition, U.S. Patent No. 2,921,027 discloses the use of oxyethylated . sorbitan mono-esters. The actual products employed are "Tweens" specifically Tween and Tween 81, both being mono-esters which only differ in their degree of oxyethylation. Anticorrosion properties are demonstrated using the "static water-drop test" and it is made absolutely plain that only the polyoxyethylene sorbitan monooleates meet the requirements of this test. Indeed, the disclosure of this U.S. Patent is very definite in its teaching of the use of monoesters, the only thing being varied being the degree of oxyethylation of such esters.

The present invention is founded upon the unexpected discovery, that the rust and corrosion-inhibiting properties of lubricating oil are significantly improved by addition of the combination of an oxyalkylated sorbitan tri-fatty acid ester, an oxyalkylated alkylphenol, especially an oxyethylated alkyl phenol, and an overbased metal detergent.

Accordingly, the present invention provides a lubricating oil composition formulated for use as a motor oil in the crankcase of an internal combustion engine comprising a lubricating oil and a corrosion-inhibiting additive characterised in that the composition comprises as additives for corrosion-inhibiting purposes an oxyalkylated sorbitan triester of a fatty acid in an amount of from 0.005 to 0.3 weight percent based on the total weight of the composition, an oxyethylated alkylphenol in an amount of from 0.01 to 0.5 weight percent based on the weight of the composition, and an overbased metal detergent.

The oxyalkylated sorbitan triester can be made by esterifying one mole of sorbitan with about three moles of fatty acid. Preferred fatty acids contain about 10-20 carbon atoms. Examples of these are decanoic acid, lauric acid, palmitic acid, stearic acid, arachidic acid, tall oil acids and the like. The most preferred fatty acid is oleic acid or mixtures of fatty acids containing substantial amounts of oleic acid.

Esterification can be conducted by known methods such as by heating a mixture of sorbitan and fatty acid to distill out water. A distillation aid such as xylene can be used. The reaction forms a mixture in which the principal component is the triester although minor amounts of di- and tetraester might form. These will not interfere with the effectiveness of the product.

The sorbitan triester is then reacted with an alkylene oxide such as ethylene oxide, propylene oxide or butylene oxide. The alkylene oxide reacts mainly with the free hydroxyl group on the sorbitan triester to form an oxyalkylene chain with a terminal hydroxyl group. The length of the chain can be varied by adjusting the ratio of alkylene oxide to sorbitan tri-fatty acid ester. Some of the alkylene oxide can react with the ester bond to insert oxyalkylene units between the sorbitan and the fatty acid. Preferably, the reaction is conducted until about 4-50 moles of alkylene oxide are reacted per mole of sorbitan tri-fatty acid ester. A preferred range is about 10-30 moles of alkylene oxide and a most preferred coadditive is formed when an average of about 20 moles of alkylene oxide react per mole of sorbitan tri-fatty acid ester.

The preferred alkylene oxide is ethylene oxide which forms a chain of repeating ethyleneoxy units.

Suitable oxyalkylated sorbitan tri-fatty acid esters are available commercially. Atsurf 2822, a product of ICI United States, Inc., is an oxyethylated sorbitan trioleate containing an average of about 20 ethyleneoxy units per molecule. It is made by esterifying one mole of sorbitan with three moles of oleic acid followed by reaction with ethylene oxide. It is very effective in the present combination.

Another required component in the combination is an ethoxylated alkylphenyl. Preferably, the alkylphenol contains about 4-12 carbon atoms in the alkyl group. More preferably, the alkyl group contains about 7-12 carbon atoms such as heptylphenol, 2-ethyl- hexylphenol, decylphenol and dodecylphenol. The most preferred alkylphenol is nonylphenol.

The coadditive is made by reacting alkylphenol with ethylene oxide until the desired number of ethylenoxy groups are reacted. Preferably there are an average of about 2-10 ethyleneoxy groups per each alkylphenol. More preferably each alkylphenol has an average of about 3-5 ethyleneoxy groups per molecule. The most preferred additive is an ethoxylated nonylphenol containing an average of about 4 oxyethylene groups. Such additives are commercially available. One such additive is marketed by Monsanto Company under the name "Sterox ND".

The amount of each additive used is such that the combination provides adequate corrosion and rust protection in an internal combustion engine and is from 0.005 to 0.3 weight percent of the oxyalkylated sorbitan triester and 0.01 to 0.5 weight percent of the oxyethylated alkylphenol.

Also required in the present invention are the overbased metal detergents. These include overbased alkaline earth metal alkylbenzene sulfonates, petroleum sulfonates, phenates, salicylates and the likes. Examples of these are overbased calcium alkylbenzene sulfonate, overbased calcium petroleum sulfonate, over- based magnesium alkylbenzene sulfonate, over- based calcium salicylate, overbased calcium alkylphenate, overbased magnesium alkylphenate sulfide and the like. Overbasing methods are well known. For example, alkylbenzene sulfonic acid having an equivalent weight of about 300-2,000 can be overbased by reaction with excess calcium oxide in the presence of water and methanol followed by carbon dioxide injection. The colloidal alkaline earth metal base in these additives serve to neutralize acids in blow-by gases formed in combustion.

Coadditives may be included in a fully formulated crankcase lubricant. Examples of these are dispersants such as the polyisobutyl succinimide of ethylenepolyamine and polyisobutyl- phenol Mannich condensates with formaldehyde and ethylenepolyamine. Metal detergents such as calcium alkylbenzene sulfonate, magnesium petroleum sulfonate, calcium salicylates and calcium alkylphenate are conventionally included.

Viscosity index improvers are generally added to improve viscosity property of the formulated oil. These include the polyalkylmeth- acrylate type and the olefin copolymer type. Examples of the latter are ethylene/propylene copolymer, styrene/butadiene copolymer and the like.

Phosphosulfurized olefins can be added such as phosphosulfurized terpenes or phosphosulfurized polybutenes. These may be further reacted by steam blowing or by neutralization with alkaline earth metal bases such as barium oxide.

Phenolic antioxidants are frequently added to the oil compositions. Examples of these are 4,4' - methylenebis - (2,6 - di - tert - butylphenol); 2,6 - di - tert - butyl - 4 - dimethyl- aminomethylphenol; 4,4' - thiobis - (2,6 - di - tert - butylphenol) and the like.

Zinc salts of dihydrocarbyldithiophosphoric acid are routinely added to provide both wear and antioxidant protection. A typical example is zinc di - (2 - ethylhexyl) - dithiophosphate.

The following Example illustrates the preparation of a typical formulated oil suitable for use in an engine crankcase.

### Example 1

In a blending vessel place 1,000 gallons (3,785 litres) 150 SUS solvent refined mineral oil. To this add 100 gallons (378.5 litres) 1- decene oligomer containing mainly trimers and tetramers. Add sufficient zinc isobutylamylthio- phosphate to provide 0.07 weight percent zinc. Add overbased (TBN 300) calcium alkylbenzene sulfonate in an amount to provide 0.15 weight percent calcium. Add 30 gallons (113.55 litres) of a polylaurylmethacrylate VI improver. Add sufficient polyisobutyl succinimide of tetraethylene pentamine to provide 3 weight percent active dispersant. Add 0.03 weight percent Atsurf 2822 and 0.3 weight percent Sterox ND. Blend the oil until homogenous and package for distribution.

In many cases the additive combination of this invention is first packaged in an additive concentrate formulated for addition to lubricating oil. Thus, the invention provides an additive concentrate formulated for addition to lubricating oil characterised by a content, for corrosion-inhibiting purposes, of both an oxyalkylated sorbitan triester of a fatty acid and an oxyethylated alkylphenol. These concentrates usually contain conventional additives such as those listed above in addition to the oxyalkylated sorbitan triester and ethoxylated alkylphenol described herein. The various additives are present in a proper ratio such that when a quantity of the concentrate is added to lubricating oil the various additives are all present in the proper concentration. The additive concentrate also contains mineral oil in order to maintain it in liquid form.

The following Example illustrates formulation of an additive concentrate formulated for addition to lubricating oil to provide an effective crankcase lubricant.

### Example 2

In a blending vessel place 1199.5 lbs. (544.6 Kg) of 100 SUS mineral oil, 748 lbs. (339.6 Kg) of polyisobutyl succinimide of tetraethylene pentamine, 2352 lbs. (1067.8 Kg) of ethylene/propylene copolymer VI improver, 264.8 lbs. (120.2 Kg) of zinc di - (2 - ethylhexyl)dithiophosphate, 245 lbs. (111.23 Kg) of overbased calcium alkylbenzene sulfonate (300 TBN), 5.88 lbs. (2.67 Kg) of Atsurf 2822 and 58.8 lbs. (26.7 Kg) of Sterox ND. Blend until homogenous and then package. The addition of 2450 lbs. (1112.3 Kg) of the above concentrate to 1,000 gallons (3785 litres) of 150 SUS mineral oil will provide an effective crankcase lubricant.

Standard multi-cylinder Sequence lid tests were carried out in a fully formulated oil containing a commercial succinimide ashless dispersant, a zinc dialkyldithiophosphate, a commercial viscosity index improver, a commercial 300 TBN overbased calcium alkylbenzene sulfonate and 0.3 weight percent Sterox ND and 0.03 weight percent Atsurf 2822. In this test a rust rating of 8.5 or above is a pass. The test was conducted using two different base oils. Ratings of 8.5 and 8.7 were obtained. Both oils passed.

## Claims

1. A lubricating oil composition formulated for use as a motor oil in the crankcase of an internal combustion engine comprising a lubricating oil and a corrosion-inhibiting additive characterised in that the composition comprises as additives for corrosion-inhibiting purposes an oxyalkylated sorbitan triester of a fatty acid in an amount of from 0.005 to 0.3 weight percent based on the total weight of the composition, an oxyethylated alkylphenol in an amount of from 0.01 to 0.5 weight percent based on the weight of the composition, and an overbased metal detergent.

2. A composition as claimed in claim 1 further characterised in that the oxyethylated alkylphenol contains about 3-5 ethyleneoxy units.

3. A composition as claimed in claim 1 or claim 2 further characterised in that the oxyalkylated sorbitan triester is an oxyethylated sorbitan trioleate.

4. A composition as claimed in claim 3 further characterised in that the oxyethylated sorbitan trioleate contains about 4-50 ethyleneoxy units.

5. A composition as claimed in claim 4 further characterised in that the oxyethylated sorbitan trioleate contains about 20 ethyleneoxy units.

6. A composition as claimed in any one of claims 1 to 5 further characterised in that the oxyethylated alkylphenol is an oxyethylated C₄-₁₂ alkylphenol.

7. A composition as claimed in claim 6 further characterised in that the oxyethylated alkylphenol is an oxyethylated nonylphenol containing an average of about 4 ethyleneoxy units.

8. A composition as claimed in any one of the preceding claims further characterised in that it contains an ashless dispersant.

9. An additive concentrate formulated for addition to a lubricating oil characterised by a content, for corrosion-inhibiting purposes, of an oxyalkylated sorbitan triester of a fatty acid, an oxyethylated alkylphenol, and an overbased metal detergent; the oxyalkylated sorbitan triester optionally being as defined in any one of claims 3 to 5, the oxyethylated alkylphenol optionally being as defined in any one of claims 2, 6 or 7 and the ratio of the amount of the triester to that of the alkylphenol being in the range of from 1 to 100:30 to 1.

10. An additive concentrate formulated for addition to a lubricating oil and containing an overbased alkaline earth metal detergent and an ash less dispersant characterised in that the concentrate also contains, for corrosion-inhibiting purposes, both an oxyalkylated sorbitan triester of a fatty acid and an oxyethylated C₄₋₁₂ alkylphenol.

## Revendications

1. Composition d'huile lubrifiante formulée en vue d'être utilisée comme huile moteur dans le carter d'un moteur à combustion interne, comprenant une huile lubrifiante et un additif inhibiteur de corrosion, caractérisée en ce qu'elle renferme comme additifs en vue d'inhiber la corrosion un triester de sorbitanne oxyalkylé d'un acide gras en une quantité de 0,005 à 0,3% en poids sur la base du poids total de la composition, un alkylphénol oxyéthylé en une quantité de 0,01 à 0,5% en poids sur la base du poids de la composition et un détergent métallique rendu surbasique.

2. Composition suivant la revendication 1, caractérisée en outre en ce que l'alkylphénol oxyéthylé contient environ 3-5 motifs éthylèneoxy.

3. Composition suivant la revendication 1 ou la revendication 2, caractérisée en outre en ce que le triester de sorbitanne oxyalkylé est un trioléate de sorbitanee oxyéthylé.

4. Composition suivant la revendication 3, caractérisée en outre en ce que le trioléate de sorbitanne oxyéthylé contient environ 4-50 motifs éthylèneoxy.

5. Composition suivant la revendication 4, caractérisée en outre en ce que le trioléate de sorbitanne oxyéthylé contient environ 20 motifs éthylèneoxy.

6. Composition suivant l'une quelconque des revendications 1 à 5, caractérisée en outre en ce que l'alkylphénol oxyéthylé est un (alkyle en C₄ à C₁₂)-phénol oxyéthylé.

7. Composition suivant la revendication 6, caractérisée en outre en ce que l'alkylphénol oxyéthylé est un nonylphénol oxyéthylé contenant en moyenne environ 4 motifs éthylèneoxy.

8. Composition suivant l'une quelconque des revendications précédentes, caractérisée en outre en ce qu'elle contient un dispersant sans cendres.

9. Concentré d'additif formulé en vue de son addition à une huile lubrifiante, caractérisé en ce qu'il contient, en vue d'inhiber la corrosion, un triester de sorbitanne oxyalkylé d'un acide gras, un alkylphénol oxyéthylé et un détergent métallique rendu surbasique; le triester de sorbitanne oxyalkylé étant éventuellement tel que défini dans l'une quelconque des revendications 3 à 5, l'alkylphénol oxyéthylé étant éventuellement tel que défini dans l'une quelconque des revendications 2, 6 ou 7 et le rapport de la quantité du triester à la quantité de l'alkylphénol étant compris dans la plage de 1 à 100:30 à 1.

10. Concentré d'additif formulé en vue de son addition à une huile lubrifiante et contenant un détergent métallique alcalino-terreux rendu surbasique et un dispersant sans cendres, caractérisé en ce qu'il contient également, aux fins de l'inhibition de la corrosion, un triester de sorbitanne oxyalkylé d'un acide gras et un (alkyle en C₄ à C₁₂)-phénol oxyéthylé.

## Patentansprüche

1. Schmieröl-Zusammensetzung formuliert zur Verwendung als Moterenöl im Kurbelgehäuse einer internen Verbrennungsmaschine, enthaltend ein Schmieröl und ein korrosionshinderndes Additiv, dadurch gekennzeichnet, daß die Zusammensetzung als Additiv zur Korrosionsverhinderung einen oxalkylierten Sorbitantriester einer Fettsäure in einer Menge von 0,005 bis 0,3 Gew.-% bezogen auf das Gesamtgewicht der Zusammensetzung, ein oxäthyliertes Alkylphenol in einer Menge von 0,01 bis 0,5 Gew.-% bezogen auf das Gewicht der Zusammensetzung, und ein überbasisches Metalldetergens enthält.

2. Zusammensetzung nach Anspruch 1, dadurch gekennzeichnet, daß das oxäthylierte Alkylphenol etwa 3 bis 5 Äthylenoxy-Einheiten enthält.

3. Zusammensetzung nach Anspruch 1 oder 2, dadurch gekennzeichnet, daß der oxalkylierte Sorbitantriester ein oxäthyliertes Sorbitantiroleat ist.

4. Zusammensetzung nach Anspruch 3, dadurch gekennzeichnet, daß das oxäthylierte Sorbitantrioleat etwa 4 bis 50 Äthylenoxy-Einheiten enthält.

5. Zusammensetzung nach Anspruch 4, dadurch gekennzeichnet, daß das oxäthylierte Sorbitantrioleat etwa 20 Äthylenoxy-Einheiten enthält.

6. Zusammensetzung nach einem der Ansprüche 1 bis 5, dadurch gekennzeichnet, daß das oxäthylierte Alkylphenol ein oxäthyliertes C₄-₁₂-Alkylphenol ist.

7. Zusammensetzung nach Anspruch 6, dadurch gekennzeichnet, daß das oxäthylierte Alkylphenol ein oxäthyliertes Nonylphenol ist, welches einen Durchschnitt von etwa 4 Äthylenoxy-Einheiten enthält.

8. Zusammensetzung nach einem der vorhergehenden Ansprüche, dadurch gekennzeichnet, daß sie ein aschefreies Dispergierungsmittel enthält.

9. Additiv-Konzentrat formuliert für die Zugabe zu einem Schmieröl, gekennzeichnet durch einen Gehalt eines oxyalkylierten Sorbitantriesters einer Fettsäure, eines oxäthylierten Alkylphenols, und eines überbasischen Metalldetergens zur Korrosionsverhinderung, wobei der oxalkylierte Sorbitantriester gegebenenfalls der Definition in einem der Ansprüche 3 bis 5 entspricht, das oxäthylierte Alkylphenol gegebenenfalls der Definition in einem der Ansprüche 2, 6 oder 7 genügt, und das Verhältnis der Menge des Triesters zu der Menge des Alkylphenols im Bereich von 1 bis 100:30 bis 1 liegt.

10. Additive-Konzentrat formuliert für die Zugabe zu einem Schmieröl und enthaltend ein überbasisches Erdalkalimetall-Detergens und ein aschefreies Dispersionsmittel, dadurch gekennziechnet, daß das Konzentrat zur Korrosions-Verhinderung auch einem oxalkylierten Sorbitantriester einer Fettsäure und ein oxäthyliertes C₄₋₁₂₋Alkylphenoi enthält.
